

Aug. 26, 1952

W. A. REX

2,608,526

## COKING OF CARBONACEOUS FUELS

Filed Dec. 14, 1946



Walter A. Rex Inventor  
by L. F. Raup Attorney

UNITED STATES PATENT OFFICE

2,608,526

## COKING OF CARBONACEOUS FUELS

Walter A. Rex, Westfield, N. J., assignor to Standard Oil Development Company, a corporation of Delaware

Application December 14, 1946, Serial No. 716,409

16 Claims. (Cl. 196—56)

1

The present invention relates to the carbonization or coking of carbonaceous fuels such as heavy oil residues, asphalts, asphaltites or the like, as well as all types of coal, lignites, cellulosic materials including lignin, oil shale, tar sands, etc., to produce valuable volatile materials and coke. More particularly, the invention is concerned with an improved method and apparatus for the continuous carbonization of these fuels in the form of finely divided solids moving much like a fluid through a treating system.

Heretofore, carbonizable fuels of the type mentioned above have been converted into liquid and gaseous fuels and coke in fixed bed, low or high temperature, coking or carbonization processes. These processes either require frequent cleaning periods resulting in discontinuous operation or they involve inefficient conversion of the available carbon into heat and volatile fuels.

The operation of these processes may be made fully continuous by employing the so-called fluid solids technique in which the reactions take place in dense fluidized beds of finely divided solids maintained in a turbulent ebullient state by means of fluidizing gases. This technique has highly desirable additional advantages including greatly improved heat distribution and ease of solids handling.

It is also known that the utilization of the carbon available in the starting material may be greatly intensified when the coking is carried out in a so-called "fluid" reactor and the heat required to support the endothermic coking reaction is generated by a combustion of the carbon of the charge and supplied to the coking zone for instance in the form of sensible heat of solid combustion residue circulated to the heat-consuming carbonization or coking reaction. In this manner, it is also possible to supply the heat required for the coking reaction directly and internally to the charge undergoing coking without an undesirable dilution of the volatile carbonization products with combustion gases and without losses of valuable volatile carbonization products by combustion.

However, even this improved coking or carbonization process falls short of a full utilization of the valuable constituents of the charge in commercial operation. In order to carry the coking procedure to substantial completeness, coking times are usually required which are conducive to the craking of valuable normally liquid coking products into gases of lower value. In addition, continuous coking processes applying the fluid solids technique involve the use of dense

1

1

2

2

6  
1

10

10

1

18

1

2

highly turbulent coking beds of substantially uniform composition throughout the bed to which the charge is continuously fed and from which coke is continuously withdrawn. The coke withdrawn will, therefore, always have an average composition between that of the fresh feed and that of a completely coked or carbonized product rather than the composition of a completely coked product as it would be desirable from the point of view of process economy as well as value of the coke product for various uses.

The present invention overcomes the aforementioned difficulties and affords various additional advantages as will appear from the following description thereof read with reference to the accompanying drawing.

It is, therefore, the principal object of my invention to provide an improved process for the continuous coking or carbonization of carbonaceous fuels.

Another object of my invention is to provide an improved coking or carbonization process which combines continuous operation with short reaction times and the production of a sufficiently coked residue.

A still further object of my invention is to provide an improved coking or carbonization process of the type specified which employs the fluid solids technique.

30 A more specific object of my invention is an improved process of coking heavy oil residues, asphaltites, carbonaceous solids, etc. in continuous operation with optimum yields of valuable volatile products.

Other and further objects and advantages of my invention will appear from the following more

I have found that these objects and advantages may be accomplished, quite generally, by contacting the carbonaceous feed to be coked or carbonized with a finely divided highly turbulent mass of solids preheated at least to a coking or carbonization temperature and maintained in an elongated solids transfer line of relatively small cross section, for a time sufficient to allow for substantially complete coking or carbonization of the feed but insufficient to permit appreciable cracking of volatile products. Carbonaceous charge and heat-carrying solids are preferably passed upwardly through the transfer line coking zone. A fluidizing gas injected into a bottom portion of the transfer line serves, in combination with product vapors, to fluidize and propel the charge through the coking zone.

5 Finely divided fluidized coke and product

vapors discharge into a disengaging and/or stripping zone of enlarged cross section which is maintained below cracking temperature and wherein coke is separated from and/or stripped of, volatile coking products preferably with the aid of a stripping gas such as steam,  $\text{CO}_2$ , other inert gases, or the like. Finely divided coke, substantially free of product vapors is preferably heated by a partial combustion in a separate heating zone to the desired solids preheating temperature and returned as heat-carrying solid to the transfer line coking zone.

An elongated transfer line of relatively narrow cross section may be readily so dimensioned as to restrict the reaction time to that required for substantially complete coking at the coking temperature employed without permitting appreciable cracking. At the same time, solids back-mixing is limited to a negligible extent while full advantage may be taken of the ideal heat distribution within the fluidized mass across the cross section of the narrow coking zone. In this manner, a coke of any desired low volatile content may be withdrawn from the discharge end of the transfer line reactor.

My invention is equally suited to the coking of carbonaceous materials which are liquid at the coking temperature such as heavy oil residues, asphalts, gilsonites or the like, as to the carbonization of carbonaceous solids such as coals, oil shale, etc. In the former case I inject the preheated liquid charge into a fluidized mass of hot coke or inert solids such as sand, clay, etc. maintained in my transfer line reactor. In the latter case, the finely divided solid charge is fed to the transfer line reactor and contacted therein with fluidized hot usually carbonaceous solid obtained in the process. In both cases, complete mixing takes place immediately upon contact of the fresh charge with the hot fluidized solids in the transfer line reactor. However, greatest advantages are obtained when applying my invention to the coking of less refractory charge materials such as oil residues, asphaltites and the like which have been found to yield volatile coking products of particularly high cracking sensitivity.

In order to assure full continuity of operation, I prefer to maintain the process solids in a fluidized condition in all stages of the process including the reaction, disengaging and combustion zones. Any conventional means known in the art of fluid solids handling such as aerated standpipes, pressurized feed hoppers, mechanical conveyors, etc. may be used to convey the process solids between the individual treating zones.

Specific equipment dimensions and operating conditions depend, of course, on the characteristics of the carbonaceous feed and the quality and relative proportions of the products desired. Quite generally, satisfactory results may be obtained when using a transfer line reactor allowing for a feed residence time of about 0.5 to 15 seconds at coking temperatures of about  $850^{\circ}$ - $1400^{\circ}$  F., pressures of about 1-50 lbs. per sq. in. and superficial gas velocities of about 2-30 ft. per second for solids particle sizes of about 50-200 mesh and bed densities of about 0.1-10 lbs. per cu. ft. within the transfer line reactor. Coke disengaging and/or stripping may be carried out at a temperature level of about  $700^{\circ}$ - $1300^{\circ}$  F. and 5-25 lbs. per sq. in. pressure. The heat-carrying solids are preferably preheated to temperatures of about  $1000^{\circ}$ - $1800^{\circ}$  F. assuming a feed ratio of about 1 to 10 lbs. of heat-carrying solids supplied at the preheating temperature

to the transfer line reactor per lb. of carbonaceous charge.

Having set forth the general nature and objects, my invention will be best understood from the more detailed description hereinafter in which reference will be made to the accompanying drawing which is a partly schematic and partly diagrammatic illustration of a system suitable for carrying out a preferred embodiment of my invention.

The system illustrated by the drawing essentially comprises a transfer line reactor 10, a combination disengaging and stripping vessel 20 and a combustion zone or heater 50 whose functions and cooperation will be forthwith explained using the coking of heavy oil residues as an example. It should be understood, however, that the system illustrated may be readily adapted to the coking or carbonization of other carbonizable fuels such as asphalts, shales, coals, etc.

Referring now in detail to the drawing, heavy oil residues such as a  $17^{\circ}$  A. P. I. East Texas residuum is fed through line 1 to a preheating furnace 3 in which the feed may be preheated to a temperature of, say, about  $500^{\circ}$ - $850^{\circ}$  F. at which no appreciable coking takes place. The preheated feed leaves preheater 3 through line 4 and is injected into the lower portion of transfer line reactor 10 with the aid of a propelling and fluidizing gas such as steam,  $\text{CO}_2$ , product gas, or the like, supplied from line 5.

Transfer line reactor 10 receives, from a conventional standpipe 12 provided with control valve 14 and one or more aeration taps 16, finely divided process coke having a fluidizable particle size of about 50-200 mesh, which has been heated to a temperature of about  $1000^{\circ}$ - $1600^{\circ}$  F. in heater 50 as will appear more clearly hereinafter. In the case of a coking feed which is liquid at the coking temperature, the coke particles supplied from standpipe 12 consist of process coke deposited on a core of non-process solid such as extraneous coke, sand, clay or the like supplied to and heated in heater 50 above coking temperature during the starting period in any suitable manner known per se. For example, the extraneous finely divided solids may, during the starting period, be suspended in an air-fuel gas mixture and the suspension may be passed through line 45 into heater 50 wherein the gas mixture may be burned to heat the solids to the desired temperatures. In the course of the operation all extraneous solid matter may disappear in the form of withdrawn coke and be replaced completely by process coke.

The liquid feed, upon contact with the hot coke in reactor 10, is quickly heated to a coking or carbonization temperature of about  $850^{\circ}$ - $1200^{\circ}$  F. as a result of the excellent heat transfer characteristics of the turbulent coke mass fluidized in and propelled through reactor 10 under the influence of the fluidizing gas supplied through line 5 and the rapid evolution of product vapors. Coke formed during the coking treatment is deposited on the fluidized solids in reactor 10. The diameter and slope of reactor 10, and the feed rates of the charge, preheated solids and fluidizing gas are so chosen that the solids in reactor 10 form an ebullient fluidized mass and travel upwardly through reactor 10. The length of reactor 10 is adapted to permit a coking time of about 1 to 10 seconds so that the charge of reactor 10 discharges into vessel 20 substantially at the coking temperature which may equal or be even above the temperature of incipient crack-

ing of volatile coking products after the coking of the charge is carried to substantial completion yielding a coke substantially free of carbonizable constituents.

In order to prevent substantial cracking of volatile coking products, it is desirable to quench the turbulent mass discharging from reactor 10 immediately upon completion of the desired coking reaction. This may be accomplished, for example, by quenching the coked suspension with steam or any other suitable gas immediately upon the entry of the suspension into the enlarged section 22 of vessel 20. I may also quench the coked suspension prior to its entry into vessel 20 by introducing into an upper portion of reactor 10, e. g. through line 11 suitable amounts of a preferably liquid quenching medium such as water, liquid feed, heavy recycle slurry of solid coke in heavy product bottoms from the product recovery system, etc. or by any combination of these methods. If water or any other extraneous quenching liquid is used in this manner, it may be desirable to allow for a contact time between the coked suspension and the quenching liquid sufficient to permit vaporization of the latter.

For the specific charge here referred to, based on a feed rate of about 50-150 bbl. per hr., reactor 10 may have a diameter of 16 to 40 in., a length of 25 to 90 ft. and a slope of 20 to 90°. Assuming a feed preheating temperature of about 850° F. and an initial temperature of the heat-carrying solids of about 1200° F., good results may be obtained at superficial gas velocities within reactor 10 of about 10 to 30 ft. per second and a solids feed rate through valve 14 of about 3 to 6 lbs. per lb. of fresh charge.

A relatively dilute suspension of finely divided product coke in fluidizing gas and product vapors discharges into the upper enlarged section 22 of vessel 20, which may attain a temperature of about 800°-1100° F. As a result of the reduction of the superficial gas velocity, a substantial proportion of the suspended coke drops out and is collected in the lower section 24 which may be provided with baffles 26. A small amount of a stripping gas, preferably steam, such as about 1-5% of steam by weight of carbonaceous charge, is injected into the bottom portion of section 24 through lines 28 to strip the coke collected in section 24 of associated product vapors and simultaneously to keep the coke in a fluidized state.

A mixture of product vapors and fluidizing gas containing some entrained coke is withdrawn overhead from disengaging zone 22 and passed through conventional gas-solids separation equipment such as cyclone 30. Coke separated in cyclone 30 may be circulated through line 32 to the coke bed in stripping section 24. Product vapors and gases, now substantially free of coke, are withdrawn through line 34 to be passed to any conventional product recovery system (not shown).

In accordance with another modification of my invention, substantial cracking of volatile coking products may be prevented by introducing the coked suspension from reactor 10 through line 79 directly into cyclone 30. In this manner, the product vapors are separated immediately from the hot coke and withdrawn from hot surfaces without time being allowed for any appreciable cracking.

Stripped fluidized product coke, which is practically free of carbonizable constituents, is withdrawn downwardly from stripping zone 24

through a conventional standpipe 36 provided with control valve 38 and one or more aerating taps 40.

Fluidized coke from standpipe 36 feeds into line 45 wherein it is suspended in a combustion-supporting gas such as air and/or oxygen fed from line 43. The dilute suspension formed is passed under the pseudo-hydrostatic pressure of the fluidized coke column in standpipe 36 through line 45 into the lower conical portion 47 of heater 50 and enters the cylindrical main section of heater 50 through a foraminous distributing member such as grid 49. The solids form, in heater 50 above grid 49, a dense, turbulent, ebullient bed fluidized by the combustion-supporting gas and the gaseous combustion products.

Combustion of coke in heater 50 takes place at temperatures which may vary between 1000° and 1600° F. depending on the oxygen supply which may be readily adjusted to the heat requirements in reactor 10. Superficial gas velocities of about 0.5-1.5 ft. per second in heater 50 and an oxygen supply of about 0.07 to 0.20 lb. per lb. of heavy residue charged are generally suitable for this purpose. Flue gas is taken overhead from level L<sub>50</sub> of the fluidized heater bed and preferably passed through conventional gas-solids separation equipment such as cyclone 52. Separated coke fines may be returned through pipe 54 to the fluidized heater bed while hot flue gases substantially free of solids are withdrawn through line 56 to be put to any desired use or to be vented, preferably after a suitable heat exchange with process fluids and/or solids.

Fluidized residual coke is withdrawn downwardly from heater 50 and passed substantially at the heater temperature through standpipe 12 to reactor 10 in the proportions indicated above to supply the heat and fluidizable solids required in reactor 10. Excess coke may be recovered as product coke from heater 50 through withdrawal line 58, if desired, after suitable heat exchange with process fluids or solids, or from stripping section 24 through line 29.

As mentioned above, the system illustrated by the drawing may also be used for the carbonization of carbonaceous materials which are solid at the carbonization conditions such as all types of coals, oil shale, cellulosic materials, and the like. When such materials are used they may be supplied in a fluidizable particle size from a feed hopper 70 through a conventional standpipe 72 aerated through one or more taps 74 and provided with a control valve 76. The fluidized solids feed discharges into line 1 wherein it may be suspended in a propelling or fluidizing gas such as steam and supplied to reactor 10 to be further treated substantially as described above. The turbulent state of the solids charge of reactor 10 affords immediate and complete mixing and heat exchange with the hot solid supplied from standpipe 12.

It will be understood that standpipes 12, 36 and 72 should be high enough to exert sufficient hydrostatic pressure on their bases to overcome the pressure and frictional resistance in the direction of the contemplated flow of the solids from these standpipes through the system. Other conventional means for conveying fluidized solids such as pressurized feed hoppers, mechanical conveyors or the like may replace any or all of standpipes 12, 36 and 72. Instead of suspending the solids withdrawn from stripping zone 24 in air line 45 these solids may be fed directly and independently of the gas-supply to heater 50 in

any conventional manner. If desired, a combustion-supporting gas such as air and/or oxygen may be added to reactor 10 through line 5 or any desired place along the length of reactor 10 to generate additional heat by partial combustion within reactor 10. Other modifications of the system illustrated may appear to those skilled in the art without deviating from the spirit and scope of my invention.

My invention will be further illustrated by the following specific example.

*Example*

Feed—17.2% A. P. I. East Texas residuum:

|                                       |                            |
|---------------------------------------|----------------------------|
| Feed preheat in furnace 3             | 850° F.                    |
| Feed rate thru 4                      | 100 bbl./hr.               |
| Average temperature in reactor 10     | 990° F.                    |
| Average pressure in reactor 10        | 15 p. s. i. g.             |
| Average temperature in vessel 50      | 1200° F.                   |
| Average pressure in vessel 50         | 2 p. s. i. g.              |
| Length reactor 10                     | 60 ft.                     |
| Slope reactor 10                      | 45°                        |
| Diameter reactor 10                   | 22 in.                     |
| Average temperature vessel 22         | 850° F.                    |
| Average pressure vessel 22            | 5 p. s. i. g.              |
| Average particle size circulated coke | 40-200 microns.            |
| Coke rate thru valve 14               | 3.4# coke/# feed.          |
| Air rate thru line 43                 | 4.6 S. C. F. air/# feed.   |
| Coke rate thru valve 38               | 3.5# coke/# feed.          |
| Stripping steam thru line 28          | 1 weight percent on feed.  |
| Diameter stripping section 24         | 24 in.                     |
| Diameter disengaging section 22       | 10 ft. 9 in.               |
| Liquid quench water temperature       | 65° F.                     |
| Liquid quench water rate thru 77      | 15 weight percent on feed. |
| Steam injection thru line 5           | 3 weight percent on feed.  |

|                                  | Short Contact Time | Conventional Fluid Technique |
|----------------------------------|--------------------|------------------------------|
| Comparison of yields:            |                    |                              |
| Coking temperature, ° F          | 990                | 990                          |
| Pressure, p. s. i. g.            | 15                 | 15                           |
| Feed rate volume liquid          |                    |                              |
| Feed/volume reactor/hr.          | 3.8                | 0.30                         |
| Contact time, seconds            | 3                  | 15-25                        |
| Yields:                          |                    |                              |
| Dry gas, weight percent          | 10.7               | 15.0                         |
| Total distillate, volume percent | 82.3               | 76.0                         |
| Coke, weight percent             | 9.3                | 12.0                         |

The above data demonstrate the superiority of my invention over conventional fluid coking operation with respect to liquid product yields. In addition considerable product quality advantages accrue to my technique inasmuch as the gas oil Diesel index is consistently appreciably higher and the Conradson carbon test on the gas oil is consistently lower than those of gas oils obtained in conventional coking operation, while gasoline inspection remains unaffected.

While the foregoing description and exemplary operations have served to illustrate specific applications and results of my invention, other modifications obvious to those skilled in the art are within the scope of the invention. Only such limitations should be imposed on the invention as are indicated in the appended claims.

I claim:

1. The process of producing volatile fuels from carbonizable materials at a carbonization temperature which comprises passing carbonizable material through an elongated narrow path in contact with a mass of finely divided solids fluidized by an upwardly flowing gas and heated independently of said carbonizable material at least to said carbonization temperature, for a time of about 0.5-15 seconds sufficient to carbonize said carbonizable material substantially completely but insufficient to permit substantial cracking of volatile carbonization products to gases, controlling the flow velocity of said gas between about 2-30 ft. per second so as to maintain high turbulence of said mass across the cross-sectional area of said path and to force said gas and said mass in the same direction upwardly through said

path while preventing substantial back-mixing of solids against the flow direction of the charge, discharging fluidized solids and volatile products into a disengaging zone, withdrawing finely divided coke from said disengaging zone and withdrawing volatile carbonization products from said disengaging zone.

2. The process of claim 1 wherein said carbonizable material is liquid at said carbonization temperature.

3. The process of claim 1 wherein said carbonizable material is solid at the carbonization temperature.

4. The process of claim 1 wherein said fluidized mass of solids comprises product coke.

5. The process of producing volatile products from carbonizable fuels by subjecting said fuels to a carbonization temperature which comprises passing carbonizable material upwardly through an elongated narrow path in contact with a turbulent mass of finely divided solids fluidized by an upwardly flowing gas and heated independently of said carbonizable material at least to said carbonization temperature, for a time of about 0.5-15 seconds sufficient to carbonize said carbonizable material substantially completely to form volatile products and coke but insufficient to permit substantial cracking of volatile carbonization products to gases, controlling the flow velocity of said gas between about 2-30 ft. per second so as to maintain high turbulence of said mass across the cross-sectional area of said path and to force said gas and said mass in the same direction upwardly through said path while preventing substantial back-mixing of solids against the flow direction of the charge, discharging fluidized solids and volatile products from said path into a disengaging zone, withdrawing volatile carbonization products from said zone,

30 separately withdrawing finely divided coke from said zone, passing finely divided coke thus withdrawn to a combustion zone, subjecting finely divided coke in said combustion zone to a combustion reaction to heat said coke at least to said carbonization temperature and passing finely divided coke so heated from said combustion zone to said path at a rate sufficient to supply at least a portion of the heat of carbonization required on said path.

6. The process of claim 5 wherein said coke is stripped of associated volatile carbonization products prior to passing said coke to said combustion zone.

7. The process of claim 5 wherein said coke is subjected to said combustion reaction in a dense turbulent bed of finely divided solids fluidized by an upwardly flowing combustion-supporting gas.

8. The process of claim 5 wherein the temperature in said disengaging zone is below the incipient cracking temperature of volatile carbonization products.

9. The process of claim 5 wherein said carbonizable material is liquid at said carbonization temperature and said fluidized mass comprises a finely divided extraneous solid.

10. The process of claim 5 wherein the temperature in said disengaging zone is substantially the same as said carbonization temperature.

11. The process of claim 5 wherein said solids and volatile products in said path are quenched to a temperature below incipient cracking temperature prior to the separation of coke from volatile products.

12. In the process of continuously carbonizing carbonizable fuels in the form of a turbulent bed of fluidized solids maintained in a carbonization

zone and supplying heat of carbonization as sensible heat of finely divided product coke heated by a combustion reaction carried out in a dense fluidized bed of product coke maintained in a separate combustion zone, the improvement which comprises controlling the carbonization time at a length within about 0.5-15 seconds desirable for the prevention of cracking of volatile products to gases by passing said carbonizable material in contact with a fluidized mass of said heated coke at a controlled rate upwardly through a carbonization zone forming an inclined elongated narrow path having a ratio of length over diameter of at least 7 and a diameter adapted to permit at the prevailing flow rate turbulence of the charge across the cross-section of said path and to prevent substantial backmixing of solids against the flow direction of the charge.

13. The process of claim 12 wherein fluidized coke and carbonization products flow in the same direction upwardly through said path.

14. The process of producing volatile products from liquid carbonizable fuels of comparatively high specific gravity and high viscosity yielding volatile coking products of high cracking sensitivity, which comprises subjecting said fuels to a carbonization temperature within the range of 850° to 1200° F., passing said carbonizable fuels upwardly through an inclined elongated transfer line carbonization zone in contact with a turbulent mass of heated solids of particle size within the range of 50 to 200 mesh, fluidized by an upwardly flowing gas stream having a superficial velocity of about 2 to 30 ft. per second, to form a fluid solids mass of density 0.1 to 10 lbs. per cu. ft. and heated independently of said carbonizable material at least to said carbonization temperature, for a period of from about 0.5 to 15 seconds within said reaction zone sufficient to carbonize said carbonizable liquids substantially completely to form volatile products and coke, but insufficient to crack said volatile carbonization products to a substantial degree to gases, controlling the flow velocity of said gas between about 2-30 ft. per second so as to maintain high turbulence of said mass across the cross-sectional area of said path and to force said gas and said mass in the same direction upwardly through said path while preventing substantial back-mixing of solids against the flow direction of the charge, discharging fluidized solids and volatile products from said transfer line reaction zone into a disengaging zone, withdrawing volatile carbonization products from said zone, passing finely divided coke thus withdrawn, to a combustion zone, subjecting finely divided coke in said combustion zone to a combustion reaction to heat said coke at least to said carbonization temperature, and

passing finely divided coke so heated, from said combustion zone to said transfer line carbonization zone at a rate sufficient to supply at least a portion of the heat of carbonization required in said carbonization zone.

15. The process of producing volatile products from liquid carbonizable fuels of relatively high specific gravity and high viscosity, which comprises passing said fuels at a carbonization temperature of about 850°-1400° F. through an elongated narrow path in contact with a mass of finely divided solids fluidized by an upwardly flowing gas and heated independently of said carbonizable fuel at least to said carbonization temperature, for a time of about 0.5-15 seconds sufficient to carbonize said fuels substantially completely but insufficient to permit substantial cracking of volatile carbonization products to gases, controlling the flow velocity of said gas between about 10-30 ft. per second so as to maintain high turbulence of said mass across the cross-sectional area of said path and to force said gas and said mass in the same direction upwardly through said path while preventing substantial back-mixing of solids against the flow direction of the charge, discharging fluidized solids and volatile products into a disengaging zone, withdrawing finely divided coke from said disengaging zone and withdrawing volatile carbonization products from said disengaging zone.

16. The process of claim 15 in which said disengaging zone is a gas-solids separation zone wherein solids are separated from gas by centrifugal action, and in which said fluidized solids and volatile products are passed directly from said path into said separation zone.

WALTER A. REX.

#### REFERENCES CITED

40 The following references are of record in the file of this patent:

#### UNITED STATES PATENTS

| Number    | Name          | Date          |
|-----------|---------------|---------------|
| 1,858,834 | Lucke         | May 17, 1932  |
| 1,941,809 | McKee         | Jan. 2, 1934  |
| 1,950,558 | Karrick       | Mar. 13, 1934 |
| 2,285,276 | Hemminger     | June 2, 1942  |
| 2,301,322 | Reeves et al. | Nov. 10, 1942 |
| 2,339,932 | Kuhl          | Jan. 25, 1944 |
| 2,344,900 | Reeves        | Mar. 21, 1944 |
| 2,360,787 | Murphree      | Oct. 17, 1944 |
| 2,362,270 | Hemminger     | Nov. 7, 1944  |
| 2,412,667 | Arveson       | Dec. 17, 1946 |
| 2,412,879 | Fischer       | Dec. 17, 1946 |
| 2,414,586 | Egloff        | Jan. 21, 1947 |
| 2,436,160 | Blanding      | Feb. 17, 1948 |
| 2,439,811 | Jewell        | Apr. 20, 1948 |